

Patented Dec. 28, 1926.

1,612,453

# UNITED STATES PATENT OFFICE.

WILSON T. LUNDY AND HOMER S. BURNS, OF FREEPORT, TEXAS, ASSIGNEES TO FREEPORT SULPHUR COMPANY, OF FREEPORT, TEXAS, A CORPORATION OF TEXAS.

## PROCESS FOR MINING SULPHUR.

No Drawing.

Application filed August 5, 1926. Serial No. 127,475.

Our invention relates to the process of recovery of elemental sulphur from sulphur bearing deposits by means of what is commonly known as the hot-water method. It has for its object the better control of the movement of the fluid heating medium (commonly water) used in this process.

In order that the operation of our invention may be made clear we will first describe the nature of the sulphur bearing formations commonly encountered in the United States and will also briefly describe the so-called hot-water method as now generally applied to sulphur mining.

15 By far the greater part of the sulphur known to exist in the elemental form on the American Continent occurs in the form of pure crystals of elemental sulphur interspersed with gypsum or lime rock or mixtures of these rocks. It occurs usually in what are known as "domes," which are found in considerable numbers along the coastal plane bordering on the Gulf of Mexico in the States of Texas and Louisiana. The sulphur bearing portion of these domes, or of such of them as are known to contain sulphur, lies at depths varying from a few hundred feet up to 1500 or 2000 feet. The sulphur bearing portions of these dome formations are usually more or less porous or spongy. They contain cavities of widely varying sizes, from minute pores to cavities of very great size, which may be aptly described as caverns. These cavities are more or less inter-connected by channels through which water may circulate with a greater or less degree of freedom depending upon the number and sizes both of the cavities or pores, and of the inter-connecting channels. 40 Being at considerable depth in the ground and below the water table, these cavities, pores, channels and caverns are filled with water. This water being in contact with sulphur, limestone, gypsum and other rocks and earths, contains in solution considerable quantities of solid matter. In different sulphur bearing formations and also in different portions of the same sulphur bearing formation, there is often to be found a great degree of variation in what may be termed the permeability of the formation. This permeability is a function of and is affected by two variables. One variable 55 is the size and number of the pores or cavities in the sulphur bearing formation

and the second variable is the number and size of the inter-connecting passages or channels between the cavities. Some of the effects of this difference in permeability will be described later.

60 The recovery of sulphur from these sulphur bearing formations situated at depths of several hundred feet under the surface of the ground is commonly accomplished by what is generally known as the hot water process. This process consists essentially in forcing water at a high temperature, usually above 300° F., and under a pressure usually above 100 lbs. per square inch, into the sulphur bearing formation, and raising to the 70 surface of the ground the sulphur melted by the water.

75 In the carrying out of this process holes are drilled from the surface of the ground down into and through the sulphur producing horizon. In these holes or wells are placed a series of pipes of various diameters one within another in such a manner that hot water under the desired pressure and temperature conditions may be forced into the sulphur bearing strata through the water pipes, and also that fluid or melted sulphur may be simultaneously lifted to the surface through one of the inner pipes of the series.

80 The hot water so injected into the sulphur bearing formation moves through the pores and cavities of the formation and while so passing raises the temperature of the formation with which it comes into contact. This rise of temperature continues until those portions of the formation through which quantities of the hot water have passed reach a temperature approximately equal to that of the injected water. As pure sulphur melts at about 240° F., and as the hot water is injected at a considerably higher temperature, there results a melting of the sulphur contained in the formation. This melted sulphur, being much heavier than the water, finds its way downward through the heated portion of the porous formation surrounding the bottom and lower portion of the pipes and enters the pipes through perforations suitably placed and provided for the purpose. This molten sulphur is then lifted to the surface of the ground by means of compressed air, utilizing the well known device known as an "air lift."

85 As already stated, there is a wide difference between sulphur formations and also be-

tween different portions of the same formation as regards the permeability of the formation. In some cases the pores, cavities and passages are relatively small in size and few in number and uniformly distributed throughout the formation. In other cases these cavities are much more numerous, much larger and unevenly distributed throughout the formation. In some formations it is not uncommon to find very large cavities and very open channels through which the water may pass. In the former case, where the pores, cavities and passages are small and uniformly distributed the water may find its way slowly through the openings and radiate uniformly in all directions from the pipes through which it is injected into the sulphur bearing formation. This is a very desirable condition and results in a relatively complete melting of the sulphur in all directions from the pipes. In the latter case, where the cavities and passages are much larger and irregularly distributed, it is found that the hot water finds a free and easy passage away from the pipes through channels or openings in one or more directions and a relatively obstructed and difficult passage in other directions, the result is that only a relatively small proportion of the sulphur in the vicinity of the pipes is melted. This often results in large and valuable deposits of sulphur remaining unmelted within easy melting radius from the well after production has ceased. We have found that this quick and free passage of the melting fluid can be overcome by the use of a hot fluid of greater viscosity than plain water such as is commonly used. This viscous fluid may be prepared by mixing either soluble or insoluble solids or liquids in the water to be used as a heating medium. We have found that we can produce a suitable viscous fluid by making an intimate mixture of water with a solid and relatively insoluble substance as, for example, a very finely precipitated lime such as that produced when "hard" water is treated with caustic lime or hydrated lime to precipitate the dissolved lime from the water. This precipitated lime, commonly called "lime sludge," is a waste product of a water treating plant and is of little or no commercial value. In fact, it is usually a difficult and costly by-product to dispose of. By mixing lime sludge with water in proper proportions we produce a fluid having a relatively high viscosity. This fluid, of relatively high viscosity, is heated to a suitable temperature above the melting point of sulphur and is injected into the sulphur bearing formation in a manner similar in general to that described above. The increased viscosity of the heating fluid tends to retard the passage of the fluid through the cavities and passages of the porous sulphur bear-

ing formation, and so tends to more evenly distribute its flow in all directions from the well.

Another important feature of our invention lies in the greater resistance to the migration of the waters naturally occurring in the porous sulphur bearing formations, which is introduced by the pressure of a viscous liquid in the cavities of the formation. The filling of cavities, passages and crevices of an open, porous type of sulphur bearing formation with a viscous liquid, restricts and reduces the freedom of flow of "formation water," from one portion of the sulphur bearing horizon to another and so lessens the diffusion and dispersion of the heat carried into the formation by the fusing medium. This restricted migration of the formation water results in greater yield of melted sulphur for a given amount of fusing liquid discharged into the formation.

Still another important characteristic of our invention is the advantage to be gained by injecting our viscous fusion fluid into operating wells so that sulphur may be continually melted from a gradually increasing area surrounding the well while the molten sulphur is simultaneously being removed from the bottom of the well to the surface of the ground.

Other and further advantages of our process will appear to one skilled in the art, who applies it to the mining of sulphur.

We claim as new and novel:

1. The process of mining sulphur which consists of injecting into the sulphur bearing formation a hot fusing liquid having a viscosity greater than that of water, and recovering the fused sulphur.

2. The process of mining sulphur which consists of injecting into the sulphur bearing formation a liquid having a temperature higher than the melting point of sulphur and a viscosity greater than that of water, and recovering the fused sulphur.

3. The process of mining sulphur which consists of injecting into the sulphur bearing formation a hot aqueous solution having a viscosity greater than that of water and recovering the fused sulphur.

4. The process of mining sulphur which consists of injecting into the sulphur bearing formation a heated mixture of water and a colloidal material in suspension, said mixture having a viscosity greater than that of water, and recovering the fused sulphur.

5. The process of mining sulphur which consists of injecting into the sulphur bearing formation a heated mixture of water and precipitated calcium carbonate having a viscosity greater than that of water, and recovering the fused sulphur.

6. The process of mining sulphur which consists of injecting into the sulphur bearing formation a heated mixture of water and

70

80

85

90

95

100

110

115

120

125

130

lime sludge, said mixture having a viscosity greater than that of water, and recovering the fused sulphur.

7. The process of mining sulphur which 5 consists of injecting into the sulphur bearing formation a heated mixture of water and a finely divided earthy material, said mixture having a viscosity greater than that of water, and recovering the fused sulphur.

10 8. The process of mining sulphur which consists of injecting into the sulphur bearing formation a heated mixture of water and colloidal clay, said mixture having a viscosity greater than that of water and recovering 15 the fused sulphur.

9. The process of mining sulphur which consists of injecting into the sulphur bearing formation a heated fusing liquid consisting essentially of minute particles of insoluble 20 earthy materials in suspension in water, said fluid having a viscosity greater than that of water, and recovering the fused sulphur.

10. The process of mining sulphur which 25 consists of injecting into the sulphur bearing formation a heated mixture of "lime sludge" and water, containing not less than 20%

by weight of lime sludge and having a viscosity greater than that of water, and recovering the fused sulphur.

30 11. The process of mining sulphur which consists of injecting into the sulphur bearing formation a heated mixture of lime sludge and water, containing not less than 30% by weight of lime sludge and having a viscosity 35 greater than that of water, and recovering the fused sulphur.

12. The process of mining sulphur which consists of injecting into the sulphur bearing formation a heated fusing fluid consisting of 40 a colloidal suspension of earthy materials in water, said fluid having a viscosity greater than that of water; and recovering the fused sulphur.

45 13. The process of mining sulphur which consists of injecting into the sulphur bearing formation a hot fusion liquid having a viscosity greater than that of water, and simultaneously recovering the fused sulphur.

Signed at Freeport, in the county of Bra- 50 zoria, and State of Texas, this 19th day of July, A. D., 1926.

WILSON T. LUNDY.  
HOMER S. BURNS.